



US009410319B2

(12) **United States Patent**  
**Ziegler et al.**

(10) **Patent No.:** **US 9,410,319 B2**  
(45) **Date of Patent:** **Aug. 9, 2016**

(54) **HEAT AND PRESSURE GENERATED DESIGN**

(71) Applicant: **VALINGE INNOVATION AB**, Viken (SE)

(72) Inventors: **Goran Ziegler**, Viken (SE); **Kent Lindgren**, Perstorp (SE)

(73) Assignee: **VALINGE INNOVATION AB**, Viken (SE)

(\*) Notice: Subject to any disclaimer, the term of this patent is extended or adjusted under 35 U.S.C. 154(b) by 0 days.

(21) Appl. No.: **14/184,299**

(22) Filed: **Feb. 19, 2014**

(65) **Prior Publication Data**

US 2014/0171554 A1 Jun. 19, 2014

**Related U.S. Application Data**

(62) Division of application No. 12/976,213, filed on Dec. 22, 2010, now abandoned.

(60) Provisional application No. 61/295,550, filed on Jan. 15, 2010.

(51) **Int. Cl.**  
**E04C 2/24** (2006.01)  
**B44C 5/04** (2006.01)  
**E04F 13/08** (2006.01)

(52) **U.S. Cl.**  
CPC ..... **E04C 2/246** (2013.01); **B44C 5/0476** (2013.01); **E04F 13/0871** (2013.01); **Y10T 428/24995** (2015.04); **Y10T 428/249924** (2015.04)

(58) **Field of Classification Search**

None

See application file for complete search history.

(56)

**References Cited**

**U.S. PATENT DOCUMENTS**

|             |         |               |
|-------------|---------|---------------|
| 2,587,064 A | 2/1952  | Rapson        |
| 2,831,793 A | 4/1958  | Elmendorf     |
| 2,962,081 A | 11/1960 | Dobry et al.  |
| 3,032,820 A | 5/1962  | Johnson       |
| 3,135,643 A | 6/1964  | Michl         |
| 3,286,006 A | 11/1966 | Annand        |
| 3,308,013 A | 3/1967  | Bryant        |
| 3,325,302 A | 6/1967  | Hosfeld       |
| 3,342,621 A | 9/1967  | Point et al.  |
| 3,345,234 A | 10/1967 | Jecker et al. |
| 3,426,730 A | 2/1969  | Lawson et al. |

(Continued)

**FOREIGN PATENT DOCUMENTS**

|    |              |        |
|----|--------------|--------|
| AU | 80284/75     | 6/1975 |
| CA | 2 557 096 A1 | 7/2005 |

(Continued)

**OTHER PUBLICATIONS**

Lindgren, Kent, et al., U.S. Appl. No. 14/321,288, entitled "A Method of Manufacturing Panel and a Building Panel," filed Jul. 1, 2014.

(Continued)

*Primary Examiner* — Elizabeth A Quast

*Assistant Examiner* — Kyle Walraed-Sullivan

(74) *Attorney, Agent, or Firm* — Buchanan Ingersoll & Rooney P.C.

(57) **ABSTRACT**

A wood fiber based panel with surfaces layer with lower parts which has less binders than the upper parts. Also, a method of manufacturing a building panel having a structured surface with a design that has color variation in register with the structure obtained by a varying pressure distribution applied on the surface.

**19 Claims, 2 Drawing Sheets**



| (56)                  | References Cited |                     |                   |                   |                      |                       |            |
|-----------------------|------------------|---------------------|-------------------|-------------------|----------------------|-----------------------|------------|
| U.S. PATENT DOCUMENTS |                  |                     |                   |                   |                      |                       |            |
| 3,463,653 A           | 8/1969           | Letter              | 9,255,405 B2      | 2/2016            | Pervan et al.        |                       |            |
| 3,486,484 A           | 12/1969          | Bullough            | 9,296,191 B2      | 3/2016            | Pervan et al.        |                       |            |
| 3,533,725 A           | 10/1970          | Bridgeford          | 2001/0006704 A1   | 7/2001            | Chen et al.          |                       |            |
| 3,540,978 A *         | 11/1970          | Ames .....          | 428/325           | 2001/0009309 A1   | 7/2001               | Taguchi et al.        |            |
| 3,565,665 A           | 2/1971           | Stranch et al.      | 2002/0054994 A1   | 5/2002            | Dupre et al.         |                       |            |
| 3,673,020 A           | 6/1972           | De Jaeger           | 2002/0100231 A1   | 8/2002            | Miller               |                       |            |
| 3,846,219 A           | 11/1974          | Kunz                | 2002/0155297 A1   | 10/2002           | Shuren               |                       |            |
| 3,880,687 A           | 4/1975           | Elmendorf et al.    | 2003/0056873 A1   | 3/2003            | Nakos et al.         |                       |            |
| 3,897,185 A           | 7/1975           | Beyer               | 2003/0059639 A1   | 3/2003            | Worsley              |                       |            |
| 3,897,588 A           | 7/1975           | Nohtomi             | 2003/0102094 A1   | 6/2003            | Tirri et al.         |                       |            |
| 3,914,359 A           | 10/1975          | Bevan               | 2003/0129361 A1   | 7/2003            | Plug                 |                       |            |
| 3,961,108 A           | 6/1976           | Rosner et al.       | 2003/0208980 A1   | 11/2003           | Miller et al.        |                       |            |
| 4,052,739 A           | 10/1977          | Wada et al.         | 2004/0123542 A1   | 7/2004            | Grafenauer           |                       |            |
| 4,093,766 A           | 6/1978           | Scher et al.        | 2004/0247831 A1   | 12/2004           | Nakagawa             |                       |            |
| 4,131,705 A           | 12/1978          | Kubinsky            | 2004/0250911 A1   | 12/2004           | Vogel                |                       |            |
| 4,255,480 A           | 3/1981           | Scher               | 2005/0003099 A1   | 1/2005            | Quist                |                       |            |
| 4,313,857 A           | 2/1982           | Blount              | 2005/0079780 A1   | 4/2005            | Rowe et al.          |                       |            |
| 4,337,290 A           | 6/1982           | Kelly et al.        | 2005/0193677 A1   | 9/2005            | Vogel                |                       |            |
| 4,420,525 A *         | 12/1983          | Parks .....         | 428/156           | 2005/0252130 A1   | 11/2005              | Martensson            |            |
| 4,430,375 A           | 2/1984           | Scher et al.        | 2006/0008630 A1   | 1/2006            | Thiers et al.        |                       |            |
| 4,474,920 A *         | 10/1984          | Kyminas et al. .... | 524/386           | 2006/0024465 A1   | 2/2006               | Briere                |            |
| 4,890,656 A           | 1/1990           | Ohsumi et al.       | 2006/0032175 A1   | 2/2006            | Chen et al.          |                       |            |
| 5,034,272 A           | 7/1991           | Lindgren et al.     | 2006/0070321 A1   | 4/2006            | Au                   |                       |            |
| 5,134,026 A           | 7/1992           | Melcher             | 2006/0145384 A1   | 7/2006            | Singer               |                       |            |
| 5,206,066 A           | 4/1993           | Horacek             | 2006/0182938 A1   | 8/2006            | Oldorff              |                       |            |
| 5,246,765 A           | 9/1993           | Lussi et al.        | 2006/0183853 A1   | 8/2006            | Szczepan             |                       |            |
| 5,258,216 A           | 11/1993          | Von Bonin et al.    | 2007/0055012 A1   | 3/2007            | Caldwell             |                       |            |
| 5,266,384 A           | 11/1993          | O'Dell              | 2007/0066176 A1 * | 3/2007            | Wenstrup et al. .... | 442/415               |            |
| 5,314,554 A *         | 5/1994           | Owens .....         | 156/154           | 2007/0166516 A1   | 7/2007               | Kim et al.            |            |
| 5,422,170 A           | 6/1995           | Iwata et al.        | 2007/0184244 A1   | 8/2007            | Doehring             |                       |            |
| 5,466,511 A           | 11/1995          | O'Dell et al.       | 2007/0207296 A1   | 9/2007            | Eisermann            |                       |            |
| 5,543,193 A           | 8/1996           | Tesch               | 2007/0218260 A1   | 9/2007            | Miclo et al.         |                       |            |
| 5,569,424 A           | 10/1996          | Amour               | 2007/0224438 A1   | 9/2007            | Van Benthem et al.   |                       |            |
| 5,601,930 A           | 2/1997           | Mehta et al.        | 2007/0256804 A1   | 11/2007           | Garcis Espino et al. |                       |            |
| 5,604,025 A           | 2/1997           | Tesch               | 2008/0000417 A1   | 1/2008            | Pervan et al.        |                       |            |
| 5,609,966 A           | 3/1997           | Perrin et al.       | 2008/0032120 A1   | 2/2008            | Braun                |                       |            |
| 5,766,522 A           | 6/1998           | Daly et al.         | 2008/0090032 A1   | 4/2008            | Perrin et al.        |                       |            |
| 5,827,788 A *         | 10/1998          | Miyakoshi .....     | 442/164           | 2008/0176039 A1   | 7/2008               | Chen et al.           |            |
| 5,855,832 A           | 1/1999           | Clausi              | 2008/0263985 A1   | 10/2008           | Hasch et al.         |                       |            |
| 5,865,003 A *         | 2/1999           | Klett .....         | D06N 5/00         | 2009/0056257 A1 * | 3/2009               | Mollinger et al. .... | 52/314     |
|                       |                  |                     | 156/62.2          | 2009/0124704 A1   | 5/2009               | Jenkins               |            |
| 5,891,564 A           | 4/1999           | Schultz et al.      |                   | 2009/0135356 A1 * | 5/2009               | Ando .....            | 349/137    |
| 5,925,296 A           | 7/1999           | Leese               |                   | 2009/0139170 A1 * | 6/2009               | Thiers .....          | 52/309.1   |
| 5,942,072 A           | 8/1999           | McKinnon            |                   | 2009/0145066 A1   | 6/2009               | Pervan                |            |
| 6,036,137 A           | 3/2000           | Myren               |                   | 2009/0155612 A1 * | 6/2009               | Pervan et al. ....    | 428/498    |
| 6,103,377 A           | 8/2000           | Clausi              |                   | 2009/0208646 A1   | 8/2009               | Kreuder et al.        |            |
| 6,238,750 B1 *        | 5/2001           | Correll et al. .... | 427/521           | 2009/0294037 A1   | 12/2009              | Oldorff               |            |
| 6,468,645 B1          | 10/2002          | Clausi              |                   | 2009/0311433 A1   | 12/2009              | Wittmann              |            |
| 6,521,326 B1          | 2/2003           | Fischer et al.      |                   | 2010/0092731 A1   | 4/2010               | Pervan et al.         |            |
| 6,537,610 B1          | 3/2003           | Springer et al.     |                   | 2010/0196678 A1   | 8/2010               | Vermeulen             |            |
| 6,620,349 B1 *        | 9/2003           | Lopez .....         | 252/607           | 2010/0223881 A1   | 9/2010               | Kalwa                 |            |
| 6,666,951 B1          | 12/2003          | Kostiw              |                   | 2010/0239820 A1   | 9/2010               | Buhlmann              |            |
| 6,769,217 B2          | 8/2004           | Nelson              |                   | 2010/0291397 A1   | 11/2010              | Pervan et al.         |            |
| 6,773,799 B1          | 8/2004           | Persson et al.      |                   | 2010/0300030 A1 * | 12/2010              | Pervan et al. ....    | 52/588.1   |
| 6,803,110 B2          | 10/2004          | Drees et al.        |                   | 2010/0307675 A1   | 12/2010              | Buhlmann              |            |
| 6,926,954 B2          | 8/2005           | Shuren et al.       |                   | 2010/0307677 A1   | 12/2010              | Buhlmann              |            |
| 6,991,830 B1          | 1/2006           | Hansson et al.      |                   | 2010/0319282 A1   | 12/2010              | Ruland                |            |
| 7,022,756 B2          | 4/2006           | Singer              |                   | 2010/0323187 A1 * | 12/2010              | Kalwa .....           | B32B 33/00 |
| 7,485,693 B2          | 2/2009           | Matsuda et al.      |                   |                   |                      |                       | 428/325    |
| 7,811,489 B2          | 10/2010          | Pervan              |                   | 2010/0330376 A1   | 12/2010              | Trksak                |            |
| 8,349,234 B2          | 1/2013           | Ziegler et al.      |                   | 2011/0175251 A1   | 7/2011               | Ziegler et al.        |            |
| 8,349,235 B2          | 1/2013           | Pervan et al.       |                   | 2011/0177319 A1   | 7/2011               | Ziegler et al.        |            |
| 8,419,877 B2          | 4/2013           | Pervan et al.       |                   | 2011/0177354 A1   | 7/2011               | Ziegler et al.        |            |
| 8,431,054 B2          | 4/2013           | Pervan et al.       |                   | 2011/0189448 A1   | 8/2011               | Lindgren et al.       |            |
| 8,480,841 B2          | 7/2013           | Pervan et al.       |                   | 2011/0189471 A1   | 8/2011               | Ziegler               |            |
| 8,481,111 B2          | 7/2013           | Ziegler et al.      |                   | 2011/0247748 A1   | 10/2011              | Pervan et al.         |            |
| 8,617,439 B2          | 12/2013          | Pervan et al.       |                   | 2011/0250404 A1   | 10/2011              | Pervan et al.         |            |
| 8,663,785 B2          | 3/2014           | Ziegler et al.      |                   | 2011/0262720 A1 * | 10/2011              | Riebel et al. ....    | 428/195.1  |
| 8,728,564 B2          | 5/2014           | Ziegler et al.      |                   | 2011/0283642 A1   | 11/2011              | Meirlaen et al.       |            |
| 8,784,587 B2          | 7/2014           | Lindgren et al.     |                   | 2011/0283650 A1   | 11/2011              | Pervan et al.         |            |
| 8,920,874 B2          | 12/2014          | Ziegler et al.      |                   | 2011/0293823 A1   | 12/2011              | Bruderer et al.       |            |
| 8,920,876 B2          | 12/2014          | Vetter et al.       |                   | 2011/0293906 A1   | 12/2011              | Jacobsson             |            |
| 8,993,049 B2          | 3/2015           | Pervan              |                   | 2012/0263878 A1   | 10/2012              | Ziegler et al.        |            |
| 9,085,905 B2          | 7/2015           | Persson et al.      |                   | 2012/0263965 A1   | 10/2012              | Persson et al.        |            |
| 9,181,698 B2          | 11/2015          | Pervan et al.       |                   | 2012/0264853 A1   | 10/2012              | Ziegler et al.        |            |

(56)

## References Cited

## U.S. PATENT DOCUMENTS

|                 |         |                 |    |               |         |
|-----------------|---------|-----------------|----|---------------|---------|
| 2012/0288689 A1 | 11/2012 | Hansson et al.  | EP | 2 105 320 A1  | 9/2009  |
| 2012/0308774 A1 | 12/2012 | Persson et al.  | EP | 2 106 903 A1  | 10/2009 |
| 2013/0092314 A1 | 4/2013  | Ziegler et al.  | EP | 2 213 476 A1  | 8/2010  |
| 2013/0095315 A1 | 4/2013  | Pervan et al.   | EP | 2 226 201 A1  | 9/2010  |
| 2013/0111845 A1 | 5/2013  | Pervan et al.   | EP | 2 246 500 A2  | 11/2010 |
| 2013/0189534 A1 | 7/2013  | Pervan et al.   | EP | 2 264 259 A2  | 12/2010 |
| 2013/0269863 A1 | 10/2013 | Pervan et al.   | FR | 2 873 953 A1  | 2/2006  |
| 2013/0273244 A1 | 10/2013 | Vetter et al.   | GB | 984 170 A     | 2/1965  |
| 2013/0273245 A1 | 10/2013 | Ziegler et al.  | GB | 1090450       | 11/1967 |
| 2014/0044872 A1 | 2/2014  | Pervan          | GB | 2 248 246 A   | 4/1992  |
| 2014/0075874 A1 | 3/2014  | Pervan et al.   | JP | 2-229002 A    | 9/1990  |
| 2014/0178630 A1 | 6/2014  | Pervan et al.   | JP | 11-291203 A   | 10/1999 |
| 2014/0188610 A1 | 7/2014  | Pervan          | JP | 2001-287208 A | 10/2001 |
| 2014/0199558 A1 | 7/2014  | Pervan et al.   | JP | 2003-311717 A | 11/2003 |
| 2014/0234531 A1 | 8/2014  | Ziegler et al.  | JP | 2003-311718 A | 11/2003 |
| 2015/0017461 A1 | 1/2015  | Lindgren et al. | JP | 2005-034815 A | 2/2005  |
| 2015/0079280 A1 | 3/2015  | Vetter et al.   | JP | 2005-074682 A | 3/2005  |
| 2015/0093502 A1 | 4/2015  | Ziegler et al.  | JP | 2005-170016 A | 6/2005  |
| 2015/0111055 A1 | 4/2015  | Persson et al.  | JP | 2005-219215 A | 8/2005  |
| 2015/0159382 A1 | 6/2015  | Pervan          | JP | 3705482 B2    | 10/2005 |
| 2015/0197942 A1 | 7/2015  | Pervan et al.   | JP | 2005-307582 A | 11/2005 |
| 2015/0197943 A1 | 7/2015  | Ziegler et al.  | JP | 2007-216692 A | 8/2007  |
| 2015/0275526 A1 | 10/2015 | Persson et al.  | JP | 2007-268843 A | 10/2007 |
| 2015/0298433 A1 | 10/2015 | Kalwa           | JP | 2008-188826 A | 8/2008  |
| 2016/0031189 A1 | 2/2016  | Pervan et al.   | NZ | 225556 A1     | 2/1992  |

## FOREIGN PATENT DOCUMENTS

|    |                    |         |    |                   |         |
|----|--------------------|---------|----|-------------------|---------|
| CH | 298894 A           | 5/1954  | WO | WO 01/00409 A1    | 1/2001  |
| DE | 1 815 312 A1       | 7/1969  | WO | WO 01/48333 A1    | 7/2001  |
| DE | 7148789 U          | 4/1972  | WO | WO 01/64408 A1    | 9/2001  |
| DE | 29 39 828 A1       | 4/1981  | WO | WO 01/68367 A1    | 9/2001  |
| DE | 33 34 921 A1       | 4/1985  | WO | WO 01/92037 A2    | 12/2001 |
| DE | 42 36 266 A1       | 5/1993  | WO | WO 02/42167 A2    | 5/2002  |
| DE | 202 14 532 U1      | 2/2004  | WO | WO 02/42373 A1    | 5/2002  |
| DE | 103 31 657 A1      | 2/2005  | WO | WO 03/078761 A1   | 9/2003  |
| DE | 20 2004 003 061 U1 | 7/2005  | WO | WO 03/095202 A1   | 11/2003 |
| DE | 10 2004 050 278 A1 | 4/2006  | WO | WO 2004/042168 A1 | 5/2004  |
| DE | 20 2006 007 797 U1 | 8/2006  | WO | WO 2004/050359 A1 | 6/2004  |
| DE | 10 2005 046 264 A1 | 4/2007  | WO | WO 2004/067874 A2 | 8/2004  |
| DE | 10 2006 024 593 A1 | 12/2007 | WO | WO 2005/054600 A1 | 6/2005  |
| EP | 0 129 430 A2       | 12/1984 | WO | WO 2005/066431 A2 | 7/2005  |
| EP | 0 129 430 B1       | 1/1990  | WO | WO 2005/080096 A2 | 9/2005  |
| EP | 0 355 829 A2       | 2/1990  | WO | WO 2005/097874 A2 | 10/2005 |
| EP | 0 611 408 A1       | 12/1993 | WO | WO 2005/116337 A1 | 12/2005 |
| EP | 0 592 013 A2       | 4/1994  | WO | WO 2005/116361 A1 | 12/2005 |
| EP | 0 656 443 A1       | 6/1995  | WO | WO 2006/007413 A1 | 1/2006  |
| EP | 0 611 408 B1       | 9/1996  | WO | WO 2006/013469 A1 | 2/2006  |
| EP | 0 732 449 A1       | 9/1996  | WO | WO 2006/015313 A2 | 2/2006  |
| EP | 0 744 477 A2       | 11/1996 | WO | WO 2006/042651 A1 | 4/2006  |
| EP | 0 914 914 A2       | 5/1999  | WO | WO 2006/043893 A1 | 4/2006  |
| EP | 0 732 449 B1       | 8/1999  | WO | WO 2006/066776 A2 | 6/2006  |
| EP | 0 744 477 B1       | 1/2000  | WO | WO 2006/126930 A1 | 11/2006 |
| EP | 1 035 255 A1       | 9/2000  | WO | WO 2007/015669 A2 | 2/2007  |
| EP | 1 125 971 A1       | 8/2001  | WO | WO 2007/042258 A1 | 4/2007  |
| EP | 1 136 251 A2       | 9/2001  | WO | WO 2007/059294 A2 | 5/2007  |
| EP | 1 193 288 A1       | 4/2002  | WO | WO 2008/004960 A2 | 1/2008  |
| EP | 1 209 199 A1       | 5/2002  | WO | WO 2008/004960 A8 | 1/2008  |
| EP | 1 242 702 A1       | 9/2002  | WO | WO 2008/148771 A1 | 12/2008 |
| EP | 1 249 322 A1       | 10/2002 | WO | WO 2009/065768 A1 | 5/2009  |
| EP | 1 454 763 A2       | 9/2004  | WO | WO 2009/065769 A2 | 5/2009  |
| EP | 1 242 702 B1       | 11/2004 | WO | WO 2009/065769 A3 | 5/2009  |
| EP | 1 498 241 A2       | 1/2005  | WO | WO 2009/065772 A1 | 7/2009  |
| EP | 1 507 664 A1       | 2/2005  | WO | WO 2009/080813 A1 | 7/2009  |
| EP | 1 507 664 B1       | 2/2005  | WO | WO 2009/116926 A1 | 9/2009  |
| EP | 1 584 378 A1       | 10/2005 | WO | WO 2009/124704 A1 | 10/2009 |
| EP | 1 681 103 A2       | 7/2006  | WO | WO 2010/084466 A2 | 7/2010  |
| EP | 1 690 603 A1       | 8/2006  | WO | WO 2010/087752 A1 | 8/2010  |
| EP | 1 847 385 A1       | 10/2007 | WO | WO 2010/094500 A1 | 8/2010  |
| EP | 1 961 556 A1       | 8/2008  | WO | WO 2011/087422 A1 | 7/2011  |
| EP | 1 985 464 A1       | 10/2008 | WO | WO 2011/087423 A1 | 7/2011  |
| EP | 1 997 623 A1       | 12/2008 |    |                   |         |
| EP | 2 025 484 A1       | 2/2009  |    |                   |         |
| EP | 1 454 763 B1       | 8/2009  |    |                   |         |

(56)

**References Cited**

## FOREIGN PATENT DOCUMENTS

WO WO 2011/129757 A1 10/2011  
WO WO 2011/141851 A2 11/2011  
WO WO 2012/004699 A2 1/2012

## OTHER PUBLICATIONS

Le Fur, X., et al., "Recycling melamine-impregnated paper waste as board adhesives," published online Oct. 26, 2004, pp. 419-423, vol. 62, Springer-Verlag, DE.  
Odian, George, "Principles of Polymerization," 1991, 3<sup>rd</sup> Edition, 5 pages incl. pp. 122-123, John Wiley & Sons, Inc., New York, NY, USA.  
Persson, Hans, et al., U.S. Appl. No. 14/516,957, entitled "Method of Manufacturing a Building Panel," filed Oct. 17, 2014.  
Vetter, Georg, et al., U.S. Appl. No. 14/553,196, entitled "Method for Producing a Building Panel," filed Nov. 25, 2014.  
Ziegler, Göran, et al., U.S. Appl. No. 14/563,167, entitled "Bright Coloured Surface Layer," filed Dec. 8, 2014.  
Kalwa, Norbert, U.S. Appl. No. 14/789,339 entitled "Panel, Use of a Panel, Method for Manufacturing a Panel and a Prepreg," filed Jul. 1, 2015.  
Pervan, Darko, et al., U.S. Appl. No. 14/980,638 entitled "Wood Fibre Based Panels with a Thin Surface Layer," filed Dec. 28, 2015.  
Pervan, Darko, et al., U.S. Appl. No. 15/061,303 entitled "Powder Overlay," filed Mar. 4, 2016.  
"Hex Netting—Fencing—Ace Hardware," from <http://www.acehardware.com/family/index.jsp?categoryId=1260278>, archived on Nov. 1, 2009, accessed through the Internet Archive, WaybackMachine, 3 pages.

International Search Report (Form PCT/ISA/210) issued in corresponding PCT/SE2010/051475, Apr. 20, 2011, 4 pages, ISA/Swedish Patent Office, Stockholm, SE.

Parquet International, "Digital Printing is still an expensive process," Mar. 2008, cover page/pp. 78-79, [www.parkettmagazin.com](http://www.parkettmagazin.com).

Floor Daily, "Shaw Laminates: Green by Design," Aug. 13, 2007, 1 pg, Dalton, GA.

Engstrand, Ola (Contact)/Valinge Innovation, Technical Disclosure entitled "Fibre Based Panels With a Wear Resistance Surface," Nov. 17, 2008, IP.com No. IPCOM000176590D, IP.com PriorArtDatabase, 76 pages.

Engstrand, Ola (Contact)/Valinge Innovation, Technical Disclosure entitled "WFF Embossing," May 15, 2009, IP.com No. IPCOM000183105D, IP.com PriorArtDatabase, 36 pages.

BTLSR Toledo, Inc. website. <http://www.bltresins.com/more.html>. "Advantages to Using Powdered Resins," May 26, 2007, 2 pages, per the Internet Archive WayBackMachine.

Nimz, H.H., "Wood," Ullmann's Encyclopedia of Industrial Chemistry, published online Jun. 15, 2000, pp. 453-505, vol. 39, Wiley-VCH Verlag GmbH & Co. KGaA, Weinheim, DE.

Pervan, Darko, et al., U.S. Appl. No. 14/151,973, entitled "Method of Producing a Building Panel and a Building Panel," Jan. 10, 2014.

Pervan, Darko, U.S. Appl. No. 14/237,617, entitled "Panel Coating," filed Feb. 7, 2014.

Pervan, Darko, et al., U.S. Appl. No. 14/192,169, entitled "Fibre Based Panels with a Wear Resistance Surface", filed Feb. 27, 2014.

Ziegler, Göran, et al., U.S. Appl. No. 14/247,839, entitled A Powder Mix and a Method for Producing a Building Panel, filed Apr. 8, 2014.

\* cited by examiner

Fig. 1



*Fig. 2*

## 1

## HEAT AND PRESSURE GENERATED DESIGN

## CROSS REFERENCE TO RELATED APPLICATIONS

The present application is a divisional of U.S. application Ser. No. 12/976,213, filed on Dec. 22, 2010, which claims the benefit of U.S. Provisional Application No. 61/295,520, filed on Jan. 15, 2010, and claims the benefit of Swedish Application No. 1050040-3, filed on Jan. 15, 2010. The entire contents of each of U.S. application Ser. No. 12/976,213, U.S. Provisional Application No. 61/295,520 and Swedish Application No. 1050040-3 are hereby incorporated herein by reference.

## TECHNICAL FIELD

The disclosure generally relates to the field of fibre-based panels with wear resistant surfaces for building panels, preferably floor panels. The disclosure relates to building panels with such wear resistance surface and to production methods to produce such panels.

## BACKGROUND

Laminate flooring typically consists of layers of different materials that are compressed under heat to form a laminated board. The typical layers are an aluminum oxide containing melamine resin impregnated alfa cellulose paper, a melamine resin impregnated printed decorative paper, a wood fibre based carrier board (HDF) and a melamine resin impregnated balancing paper. Product designs are typically made by embossing the laminated product with a structured plate or paper during the press operation, and by printing the decorative paper with different designs and colors. At typical process conditions the depth of the structuration is typically less than 0.2 mm in order to yield proper looking products. Deeper structures tend to give crazing of the surface due to insufficient pressure in parts of the board area and the limitation of stretching of the paper layers. In order to give an even more natural looking product, the printed paper and the embossed structure can be coordinated giving products that are known in the field as embossed in register (EIR).

Wood Fibre Floor (WFF) is a new type of flooring product, disclosed in WO2009/065769, the entire contents of which are hereby incorporated by reference, that includes one or more layers of substantially homogenous powder mixtures that are heat compressed in processes akin to the processes used for making laminate floors. The homogenous powder mixtures typically include fibres such as wood fibres, polymer, such as melamine formaldehyde resin, hard particles, such as aluminum oxide particles and decorative materials, such as pigment particles, minerals and fibres. WFF products have a benefit over laminate floors as no papers with limited stretch capability are present, thus very deep structures can be made without yielding the observed crazing of the surface. While under heated compression the WFF powder mixture is almost liquid like in the sense that the composition flows under pressure to fill out the crevices in the structure.

## SUMMARY OF THE INVENTION

In WFF, just as in laminate flooring, it is of great interest to make natural looking products by having for example products that have color variations matching the structure variation. It has surprisingly been found that such products can be obtained in WFF by heat and pressure variations, giving the

## 2

possibility to tailor the design in a controlled manner. Several methods to control the design are disclosed below.

By applying a pressure with an uneven distribution over the surface of a layer and given a fluidity of the layer, when the pressure is applied, which is sufficiently high, it is possible to cause parts of the composition in the layer to be displaced to the desired location. The fluidity can be increased by, for example, increasing the amount of the binder in the surface layer. The binder is preferably a melamine resin but other resins and binders may also be used.

This makes it possible to create and control the colour variation and match it with structure variations.

Control by formulation—By controlling the composition of the WFF powder mixture, such as the amount and/or type of polymer resin, such as melamine resin, the fluidity of the composition can be controlled to give more or less pressure difference (and thus more or less displacement) in the different parts of the surface during heat compression. Compositions giving a low pressure difference over the surface cause the substantially homogenous powder mixture to stay substantially homogenous giving a homogenous coloration over the surface. Compositions giving a higher pressure difference restrict the bulk powder fluidity and the homogeneity of the mixture will then be broken as the more fluid parts of the composition partially flow away. The result is a gradient of composition over the surface area. Thus, a color variation can be attained or avoided depending on the preference of the producer.

Other ways to change the fluidity of the composition is to alter the amount and/or type of fiber, use of processing aids such as plasticizers, solvents, reactive solvents and the like.

Control by heat—The typical WFF formulation consists partially of wood fibres. Such wood fibres are prone to darkening upon heating. By applying more or less heat over the surface the coloration can be controlled.

Control by pressure—Controlling the applied pressure in the heat-compressed state can also control the color difference. At higher pressure the bulk powder fluidity is restricted so the homogeneity of the powder mixture will be broken as described above to give a gradient in composition over the surface area.

Control by press plate design—By optimizing the surface area of the structure plate or paper, increased and/or decreased flow can be controlled, thus aiding in the control of color difference over the surface area.

Control by scattering, heterogeneous scattering—WFF powder can be scattered in a heterogeneous (non-uniform) way in order to provoke pressure difference over the surface area when the product is heat compressed. This can be sought after to make a local reinforcement such as in the parts of the board in which a locking element can be positioned. In such a case, the mechanical, chemical and water resistance can be optimized in the areas of the locking system that can be subjected to moisture, cleaning agents and mechanical wear.

Heterogeneous scattering can also be made to follow the structuration of the embossing plate or paper. In this case, the pressure difference can be matched to yield a product having an equal amount of material over the surface area giving equally good product properties and appearance over the surface.

Heterogeneous scattering can be used to enrich the amount of material in the protruding parts of the structure, so as to make increased chemical and mechanical properties in those parts of the surface that are subjected to the most stress from walking and cleaning.

Heterogeneous scattering can also be used to introduce differences in pressure over the area during heat compressing

in excess of what is granted from the structuration of the press plate or paper. In this case, depending on the control of the bulk fluidity of the powder mixture, color variation can be controlled.

By employing more than one powder mixture the heterogeneous scattering can have a specific formulation tailored for the application. If a protruding part should be protected, this part can be richer in resins and wear particles compared to the bulk of the product, thus saving cost of the formulation. If water resistance of a locking system area should be optimized a more hydrophobic powder mixture can be used. If a specific decorative effect is sought, the powder fluidity can be optimized to give big color variation. Choice of pigment or other design material in the heterogeneous scattering can also be used.

Control by mechanical design—Removal or surface mixing of part of the scattered powder layer by means of blowing, sucking, brushing, scraping, cutting or equivalent are also means to introduce difference of pressure over the area during heat compression. In this case, similar effects of color variation due to pressure differences can be obtained as described above for heterogenous scattering. In the case of two or more powder layers being scattered on the surface, the effect of the partial removal or mixing can be further enhanced by, for example, differences in composition of the powder layers. A local mixing, micro mixing, of powders will cause a gradient in colorations that is further enhanced by the provoked pressure difference giving a further gradient in shading of the differently colored surface. The result is a possibility to make very complex color variations over the surface.

Partial removal or surface mixing as well as inhomogeneous scattering can easily be made using robots in order to either make the design actions in a controlled or uncontrolled way so as to give either identical or individual designs.

The control methods above can be used to tailor the properties of the product. As an example, an increased wear resistance might be desired on parts of the surface.

A first aspect of the invention is a building panel comprising a decorative surface layer **5** connected to a core **6**. The surface layer is a mix comprising fibres **14**, colour substance preferably colour pigments, a binder and wear resistant particles **12**. Furthermore the surface layer comprises lower parts and upper parts and there is preferably a binder concentration gradient between the lower parts and upper parts. In a preferred embodiment the lower parts comprise less binder than the upper parts. The binder is in a preferred embodiment a resin.

A reversed condition could also be used. Having higher binder content in the lower part gives a gradient of flow to both the board and the upper part that can make it possible to have a saturated surface area between the board and the lower part.

The surface layer preferably has a substantially homogenous distribution of the wear resistant particles throughout the thickness of the layer and wear resistant particles are present from the bottom, and thereby in contact with the core, to the top.

The surface layer may in one embodiment comprise a sub layer and a top layer. The sub layer may not include wear resistant particles and colour pigments. In this case the sub layer can be considered as a scattered core.

Preferred embodiments of the first aspect of the invention are disclosed under Detailed Description of Embodiments and in the dependent product claims below.

A second aspect of the invention is a method of manufacturing a building panel having a structured surface with a design that comprises colour variation in register with the structure whereby the method comprises the steps of:

applying a layer comprising a mix of fibres, binder, preferably a resin, wear resistant particles, preferably alu-

minium oxide, and a colour substance, preferably colour pigments, on a carrier wherein the mix is floatable under heat and pressure

applying heat and pressure on the mix by a structured matrix comprising protrusions and cavities such that a controlled floating of the mix is obtained by the varying pressure distribution applied on the surface. In a preferred embodiment the resin content in the layer is adapted to the pressure such that a sufficient floating is obtained and preferably the binder is a resin and the weight content of the resin is at least 40% of the layer.

In order to increase the fluidity, the mass ratio between resins and fibres is preferably in the range of about 130-240%, more preferably in the range of 150-220%, most preferably in the range of about 180-200%. In the most preferred embodiment the mass ratio between resins and fibres is about 190%.

Preferred embodiments of the second aspect of the invention are disclosed under Detailed Description of Embodiments and in the dependent method claims below.

In order to increase the releasability, i.e., the ability to be released from and not stick to the press plate, a mass ratio between resins and the sum of the masses of the fibres and the coloring substances is preferably higher than about 60%, more preferably higher than about 100% and most preferably in the range of about 100-130%.

The layer in the method preferably has a substantially homogenous distribution of the wear resistant particles throughout the thickness of the layer and wear resistant particles are present from the bottom, and thereby in contact with the carrier, to the top.

Another aspect of the invention is to use the principles and control methods above to create a surface with even colour distribution and/or properties. In this case a layer with a fluidity, when the pressure is applied is used, that is sufficiently low, to maintain the substantially homogenous mix or substantially homogenous mix and distribution of the component in the layer. Such low fluidity can be obtained by having certain ratios between resins, fibres and pigments. One ratio could be calculated through dividing the mass of resins and the mass of fibres, this ratio is preferably less than about 90% and even more preferably less than about 80%.

Another ratio could be between the mass of resins and the sum of the mass of fibres and the mass of coloring substances; this ratio is preferably higher than about 60% and in a preferred range of about 100-130%.

#### BRIEF DESCRIPTION OF THE DRAWINGS

The following disclosure will be described in connection to preferred embodiments and in greater detail with reference to the appended exemplary drawings, wherein

FIG. 1 Illustrates a Wood Fibre Floor panel, and  
FIG. 2 Illustrates a Wood Fibre Floor panel with registered embossing according to one embodiment of the invention.

#### DETAILED DESCRIPTION OF EMBODIMENTS

FIG. 1 shows a Wood Fibre Floor (WFF) panel of the type disclosed in WO 2009/065769, where the surface layer **5** has been formed on a core **6** that has been produced in a prior separate operation, for example a HDF panel. The surface layer comprises wood fibres **14**, wear resistance particles **12** and a binder. The surface layer **5** includes an upper part **7** and a lower part **8**. The surface layer may in one embodiment comprise a sub layer and a top layer. This sub layer could be produced in the same way as the top layer and the same material compositions could be used except for the fact that in some embodiments wear resistant particles and colour pigments are not included. In this case the sub layer can be considered as a scattered core.

## 5

FIG. 2 shows one embodiment of a Wood Fibre Floor (WFF) panel according to the invention with colour variation 3 in register with the structure 2 of the surface layer 5.

Preferably the same scattering and pressing units as disclosed in WO 2009/065769 are used preferably together with a structured press plate in the method according to the invention. The panels according to the invention are preferably produced by this method.

In order to illustrate the effects of the parameters used in the control methods above, some examples are given below.

Examples 1-3 show the effect of changing the composition. Example 4 shows comparing with example 1 the effect of changing the pressure. The surface layer in Examples 1-4 is scattered in one layer. In Examples 5-6 the surface layer comprises a sub layer and a top layer. The surface layer is in all examples scattered on a HDF panel. Aluminium oxide is used as the wear resistant particles in all examples and the coloring substance is a pigment of Titanium Dioxide or combinations of Titanium Dioxide and Carbon Black.

## EXAMPLE 1

High Structure, Normal Pressure

Scattered amount: 600 g/m<sup>2</sup>  
Carrier board: 8 mm HDF  
Backing: 2 layers of NKR 140  
Structure plate: 0.7 mm Slate Structure  
Pressure: 45 kg/cm<sup>2</sup>,  
Contact time: 25 sec  
Press plate temperature: 160° C.

One Surface Layer—Scattered Homogenously

| Component                                | Wt-% |
|------------------------------------------|------|
| Melamine Formaldehyde resin              | 33   |
| Wood Fibre                               | 43   |
| Wear Resistant Particles: Aluminum Oxide | 13   |
| Coloring Substance: Titanium Dioxide     | 11   |
| Sum                                      | 100  |

The mass ratio between Melamine Formaldehyde Resin and dry components (Wood Fibre,

Coloring Substance) is equal to 61%. The mass ratio between Melamine Formaldehyde Resin and Wood Fibre is equal to 77%. The resulting product is a homogenous off white product.

## EXAMPLE 2

High Structure, Normal Pressure

Scattered amount: 600 g/m<sup>2</sup>  
Carrier board: 8 mm HDF  
Backing: 2 layers of NKR 140  
Structure plate: 0.7 mm Slate Structure  
Pressure: 45 kg/cm<sup>2</sup>,  
Contact time: 25 sec  
Press plate temperature: 160° C.

One Surface Layer—Scattered Homogenously

| Component                   | Wt-% |
|-----------------------------|------|
| Melamine Formaldehyde resin | 47   |
| Wood Fibre                  | 25   |

6  
-continued

| Component                                | Wt-% |
|------------------------------------------|------|
| Wear Resistant Particles: Aluminum Oxide | 17   |
| Coloring Substance: Titanium Dioxide     | 11   |
| Sum                                      | 100  |

The mass ratio between Melamine Formaldehyde Resin and dry components (Wood Fibre, Coloring Substance) is equal to 131%. The mass ratio between Melamine Formaldehyde Resin and Wood Fibre is equal to 188%. The resulting product is a substantially homogenous off white product with some whiter spots at the ridges of the embossed structure.

## EXAMPLE 3

High Structure, Normal Pressure

Scattered amount: 600 g/m<sup>2</sup>  
Carrier board: 8 mm HDF  
Backing: 2 layers of NKR 140  
Structure plate: 0.7 mm Slate Structure  
Pressure: 45 kg/cm<sup>2</sup>,  
Contact time: 25 sec Press plate temperature: 160° C.  
One Surface Layer—Scattered Homogenously

| Component                                | Wt-% |
|------------------------------------------|------|
| Melamine Formaldehyde resin              | 65   |
| Wood Fibre                               | 17   |
| Wear Resistant Particles: Aluminum Oxide | 11   |
| Coloring Substance: Titanium Dioxide     | 7    |
| Sum                                      | 100  |

The mass ratio between Melamine Formaldehyde Resin and dry components (Wood Fibre, Coloring Substance) is equal to 271%. The mass ratio between Melamine Formaldehyde Resin and Wood Fibre is equal to 382%. The resulting product is a substantially homogenous off white product with many whiter spots at the ridges of the embossed structure.

## EXAMPLE 4

High Structure, High Pressure

Scattered amount: 600 g/m<sup>2</sup>  
Carrier board: 8 mm HDF  
Backing: 2 layers of NKR 140  
Structure plate: 0.7 mm Slate Structure  
Pressure: 60 kg/cm<sup>2</sup>,  
Contact time: 25 sec  
Press plate temperature: 160° C.  
One Surface Layer—Scattered Homogenously.

| Component                                | Wt-% |
|------------------------------------------|------|
| Melamine Formaldehyde resin              | 47   |
| Wood Fibre                               | 25   |
| Wear Resistant Particles: Aluminum Oxide | 17   |
| Coloring Substance: Titanium Dioxide     | 11   |
| Sum                                      | 100  |

The resulting product is a substantially homogenous off white product with many whiter spots at the ridges of the embossed structure. The mass ratio between Melamine Formaldehyde Resin and dry components (Wood Fibre, Coloring

Substance) is equal to 131%. The mass ratio between Melamine Formaldehyde Resin and Wood Fibre is equal to 188%.

## EXAMPLE 5

## Heterogeneous Scattering

Scattered amount: 300+300 g/m<sup>2</sup>  
 Carrier board: 8 mm HDF  
 Backing: 2 layers of NKR 140  
 Structure plate: 0.7 mm Slate Structure  
 Pressure: 45 kg/cm<sup>2</sup>,  
 Contact time: 25 sec  
 Press plate temperature: 160° C.  
 Sub Layer Formulation—Scattered Homogenously.

| Component                                | Wt-% |
|------------------------------------------|------|
| Melamine Formaldehyde resin              | 42.2 |
| Wood Fibre                               | 28.2 |
| Wear Resistant Particles: Aluminum Oxide | 25.8 |
| Coloring Substance: Titanium Dioxide     | 3.5  |
| Coloring Substance: Carbon Black         | 0.3  |
| Sum                                      | 100  |

The mass ratio between Melamine Formaldehyde Resin and dry components (Wood Fibre, Coloring Substance) is equal to 132%. The mass ratio between Melamine Formaldehyde Resin and Wood Fibre is equal to 150%.

Top Layer Formulation—Scattered through a Shablon.

| Component                                | Wt-% |
|------------------------------------------|------|
| Melamine Formaldehyde resin              | 49.5 |
| Wood Fibre                               | 40   |
| Wear Resistant Particles: Aluminum Oxide | 10   |
| Coloring Substance: Carbon Black         | 0.5  |
| Sum                                      | 100  |

The mass ratio between Melamine Formaldehyde Resin and dry components (Wood Fibre, Coloring Substance) is equal to 122%. The mass ratio between Melamine Formaldehyde Resin and Wood Fibre is equal to 124%. The resulting product is a dark grey product with a black pattern. In the more deeply embossed regions the black color is more intense compared to the more shallow regions.

## EXAMPLE 6

## Mechanical Design

Scattered amount: 300 g/m<sup>2</sup> Sub layer+300 g/m<sup>2</sup> Top Layer  
 Carrier board: 8 mm HDF  
 Backing: 2 layers of NKR 140  
 Structure plate: 0.7 mm Slate Structure  
 Pressure: 60 kg/cm<sup>2</sup>,  
 Contact time: 25 sec  
 Press plate temperature: 160° C.  
 Sub Layer Formulation—Scattered Homogenously.

| Component                   | Wt-% |
|-----------------------------|------|
| Melamine Formaldehyde resin | 47.5 |
| Wood Fibre                  | 24.5 |

-continued

| Component                                 | Wt-% |
|-------------------------------------------|------|
| Wear Resistant Particles: Aluminium Oxide | 17.5 |
| Coloring Substance: Titanium Dioxide      | 10.5 |
| Sum                                       | 100  |

The mass ratio between Melamine Formaldehyde Resin and dry components (Wood Fibre,

Coloring Substance) is equal to 136%. The mass ratio between Melamine Formaldehyde Resin and Wood Fibre is equal to 194%.

Top Layer Formulation—Scattered Homogenously

| Component                                 | Wt-% |
|-------------------------------------------|------|
| Melamine Formaldehyde resin               | 49.5 |
| Wood Fibre                                | 40   |
| Wear Resistant Particles: Aluminium Oxide | 10   |
| Coloring Substance: Carbon Black          | 0.5  |
| Sum                                       | 100  |

The mass ratio between Melamine Formaldehyde Resin and dry components (Wood Fibre, Coloring Substance) is equal to 122%. The mass ratio between Melamine Formaldehyde Resin and Wood Fibre is equal to 124%.

After scattering of the sub layer and the top layer, a robot scratched the surface in a programmed way to remove part of the top layer.

The resulting product is a black surface having a grey-white decoration according to the action of the robot.

The invention claimed is:

1. A building panel comprising a decorative surface layer arranged on a core wherein the surface layer comprises a lower part and an upper part disposed above the lower part with a binder concentration gradient between the lower part and the upper part; the lower part of the surface layer comprises a first mix comprising fibres, coloring substance, a binder, and wear resistance particles; and the upper part of the surface layer comprises a second mix comprising the fibres, the coloring substance, the binder, and the wear resistance particles; wherein the first mix possesses a first homogenous binder concentration, and wherein the second mix possesses a second homogenous binder concentration not equal to the first homogenous binder concentration.
2. The building panel according to claim 1, wherein the lower part comprises less binder than the upper part.
3. The building panel according to claim 1, wherein the upper part comprises less binder than the lower part.
4. The building panel according to claim 1, wherein the binder is a melamine resin.
5. The building panel according to claim 1, wherein the fibres are wood fibres.
6. The building panel according to claim 1, wherein the panel is a floor panel.
7. A building panel produced according to a method of manufacturing a building panel having an evenly colored surface whereby the method comprises the steps of: applying a layer comprising a mix of fibres, binder, wear resistant particles, and a coloring substance, on a carrier wherein the mix is floatable under heat and pressure; and

applying heat and pressure on the mix,  
wherein the mass ratio between the binder and fibres is less  
than about 90%,  
wherein the layer comprises an upper part comprising a  
first mix of the fibres, the binder, the wear resistant  
particles, and the coloring substance, and the layer com-  
prises a lower part comprising a second mix of the fibres,  
the binder, the wear resistant particles, and the coloring  
substance, the upper part being disposed above the lower  
part,  
wherein the first mix possesses a first homogenous binder  
concentration, and  
wherein the second mix possesses a second homogenous  
binder concentration not equal to the first homogenous  
binder concentration.

8. The building panel according to claim 1, wherein the  
weight content of the binder is at least 40% of the surface  
layer.

9. The building panel according to claim 1, wherein the  
binders in the mix of the upper part and the lower part of the  
surface layer are provided in a powder form.

10. The building panel according to claim 1, wherein the  
surface layer has a substantially homogenous distribution of  
the wear resistant particles throughout a thickness of the  
surface layer.

11. The building panel according to claim 1, wherein the  
mass ratio between the binder and the fibres is in the range of  
130-240%.

12. The building panel according to claim 1, wherein the  
mass ratio between the binder and the fibres is in the range of  
180-200%.

13. The building panel according to claim 7, wherein the  
mass ratio between the binder and the sum of the mass of the  
fibres and the coloring substance is in the range of 100-130%.

14. A building panel comprising a decorative surface layer  
arranged on a core wherein the surface layer comprises two

5 mixes, a first mix comprising fibres, coloring substance, a  
binder and wear resistant particles, and a second mix com-  
prising fibres, coloring substance, a binder and wear resistant  
particles, wherein the first mix is applied on the second mix  
causing the first mix to be disposed above the second mix in  
the surface layer, and wherein a homogenous binder concen-  
tration of the first mix is different than a homogenous binder  
concentration of the second mix.

10 15. The building panel according to claim 14, wherein the  
content of binder in the first mix is less than the content of  
binder in the second mix.

15 16. The building panel according to claim 14, wherein the  
content of binder in the second mix is less than the content of  
binder in the first mix.

17. A building panel comprising a decorative surface layer  
connected to a core wherein the surface layer is a mix com-  
prising fibres, coloring substance, a binder and wear resistant  
particles, and

20 25 wherein the surface layer comprises a lower part and an  
upper part disposed above the lower part with a binder  
concentration gradient between the lower part and the  
upper part;  
the lower part of the surface layer comprising a first mix  
having a first homogenous binder concentration; and  
the upper part of the surface layer comprising a second mix  
having a second homogenous binder concentration not  
equal to the first homogenous binder concentration.

18. The building panel according to claim 17, wherein the  
content of binder in the first mix is less than the content of  
binder in the second mix.

19. The building panel according to claim 17, wherein the  
content of binder in the second mix is less than the content of  
binder in the first mix.

\* \* \* \* \*